

Sept. 29, 1964

G. HEINZE ETAL

3,151,041

COKING METHOD

Filed Nov. 25, 1960



1

3,151,041

## COKING METHOD

Gerald Heinze, Uferstrasse 34, Dortmund-Schoenau, Germany; Wilhelm Reerink, Meckenstockerweg 112, Essen-Bredeney, Germany; and Heinz Echterhoff, Renatastrasse 10, Essen, Germany

Filed Nov. 25, 1960, Ser. No. 76,086

Claims priority, application Germany, Nov 28, 1959,  
B 55,716; B 55,717

10 Claims. (Cl. 202—33)

The present invention relates to a coking method and particularly to a method according to which a mixture of carbonaceous briquettes and fine coal are coked together. Depending on the composition of the above mixture, particularly depending on the type and quality of fines forming a constituent of the mixture, the result of the coking process of the present invention will be either a separable mixture of the coked briquettes and of coke breeze formed of the fines constituent, or coked bodies wherein each individual coked body will consist of portions of relatively high density and of portions of relatively low density which are integral with each other, as will be explained in more detail further below.

In the past it has been proposed to produce coke briquettes by briquetting a granulated low temperature coke mixed with hard coal of high baking properties, and coking the thus-formed briquettes. Or, it has also been proposed to mix coke produced from non-baking coal with coking hard coal and tar and to form briquettes of this mixture prior to coking of the same. It has also been suggested to form mixtures of granulated coke and granulated hard coal, to briquette the mixture with or without the addition of pitch or tar and to subject the thus-formed briquettes to coking. It is furthermore known to form a mixture of coke and baking or coking hard coal, to add tar and a small quantity of water derived from low temperature carbonization thereto, thereafter to briquette and then to coke the mixture. According to another proposition, pitch or tar is used as binder for a mixture consisting of de-gassed non-coking coal and coking hard coal.

The coking of briquettes which were thus produced in various manner has been carried out in accordance with several processes known in the art as the Phurnacite, Carmaux, Brennstofftechnik, Krupp-Lurgi, Lurgi-Spuelgas, Didier and Otto Processes. Furthermore, the coking of the briquettes can also be carried out in vertical coking chambers. However, it would be most desirable to be able to produce coked briquettes in conventional horizontal by-product ovens which are readily available and which would not require any special apparatus. Experiments to produce coke briquettes in horizontal by-products ovens did not succeed, however, due to the fact that the briquettes were baked together during the coking process or were even molten together to such an extent that a mass was formed which stuck to the oven walls or tended to lock in the oven so that removal of the coked charge by pushing the same out of the oven became impossible.

Referring now to another problem which is solved according to the present invention, methods are known according to which it is possible to produce coke bodies of low or high density as desired. In these methods it is always attempted to produce coke of a definite density which varies only within relatively narrow limits. For instance regular blast furnace coke has a density of between 0.7 and 0.9 while foundry coke preferably has a density of between 0.9 and 1.1. Furthermore, there exists a variety of special purpose cokes which possess a density of between about 1.3 and 1.5. The term density is meant herein to denote "apparent density."

2

However, as will be discussed further below there appears to be a definite need for a coke product wherein each individual coke body will include, integral with each other, portions of relatively high and portions of relatively low apparent density.

It is therefore an object of the present invention to overcome the aforementioned difficulties in the production of briquetted coke.

It is another object of the present invention to provide 10 a method according to which coke briquettes can be produced in a simple and economical manner, for instance in a horizontal by-product oven.

It is a further object of the present invention to provide 15 a method for producing coke bodies each of which will consist of portions of relatively high and portions of relatively low density.

It is yet another object of the present invention to provide a simple and economical method for producing coke of controlled density, shape and composition.

Other objects and advantages of the present invention will become apparent from a further reading of the description and of the appended claims.

With the above and other objects in view, the present 25 invention contemplates a method of producing coke briquettes, comprising the steps of forming a mixture of carbonaceous briquettes which are adapted to be coked without melting together when heated under exclusion of air to between 500° and 1300° C. and of low coking fines; coking said mixture so as to transform the briquettes and the fines into coke bodies adhering to each other but slightly; and separating the thus-formed briquettes from the coked fines so as to obtain coke breeze in addition to and separated from the coke briquettes.

However, it is also within the scope of the present 30 invention to provide a method of producing coke bodies of varying density, comprising the steps of forming a mixture of carbonaceous briquettes which are adapted to be coked without melting together when heated under exclusion of air to be between 500° and 1300° C. and of strongly coking bituminous fines, and coking the mixture so as to transform the briquettes and the bituminous fines into coherent coked bodies each of which including portions of relatively high density and integral therewith portions of relatively low density.

It has been found that according to the present invention it is now possible to produce coke briquettes in any coking installation including horizontal by-product ovens by forming a mixture of fines and of such carbonaceous briquettes which when coked alone will at most superficially melt together. The mixture is then coked in conventional manner and after completion of the coking process, the thus-formed coke briquettes are separated from the coke formed of the fines. Such separation can be carried out with relatively mild mechanical means, 50 and the success of the process depends primarily on the proper choosing of the ingredients of the mixture, i.e., on the composition of the briquettes and of the fines, particularly on the properties and composition of the fines.

60 It has been proposed previously to produce a dense blast furnace coke from coal which can be coked only with difficulties, by coking such coals which contain a high proportion of volatile constituents in a mixture with briquettes made of the same type of coal. The essential difference between the method of the present invention and this prior proposition is that according to the prior art only a uniform mass of dense blast furnace coke is obtained, while according to the present invention on the one hand coke briquettes and on the other hand regular coke breeze is produced. According to the prior art process, the shape of the initial briquettes is no longer

recognizable in the finished coke product since the components of the mixture of the prior art process will completely melt together during the coking of the same.

Surprisingly, applicants have found that it is possible to coke a mixture of briquetted coal and of fines at a temperature preferably between 800° and 1300° C., without causing a melting together of the two components of the mixture and without causing a caking together of the entire coke in the coke oven. Thereby it is furthermore achieved that the coke briquettes which are formed during the process of the present invention are substantially of the same size and shape as the briquettes which form one constituent of the mixture which is subjected to coking. The slight difference in size and shape of the finished coke briquettes is due to a slight shrinkage caused by the escape of volatile constituents. A slight baking together of the briquettes and of the surrounding coke which has been formed of the fines does not cause any difficulties and in fact is desirable because it facilitates the pushing out of the coke from the coke oven. Very slight mechanical stress, for instance dressing by passing through a screening device generally will suffice for separating the coke mixture into coke briquettes and coke breeze. If necessary, this separation can be carried out by passing the mass leaving the coke oven through a coarse grinding impact grinder.

The choice of suitable fines and briquettes will primarily be determined by the coking properties of these ingredients. Preferably, the briquettes which are to be subjected to the above described coking process should be formed of non-coking coal, oxidized coal or even of coke. Only slightly baking coal may also be used or a mixture of non-baking coal with slightly or considerably baking or coking coals may be used as the material for forming the briquettes. Thus, the briquettes which are used according to the above described process may be formed of anthracite and lean coals of up to 14% volatile constituents or of coals rich in volatile constituents, preferably open-burning coals with more than 40% volatile constituents. The briquettes may also be formed of short-flaming or semibituminous coal with between 14 and 18% volatile constituents provided that such coal is only slightly coking or, if not, mixed with other slightly or not at all coking coals.

Thus, substantially all carbonaceous or coal briquettes, even those containing coke, may be used as discussed above, provided that upon heating of such briquettes under the exclusion of air to a temperature of between 500° and 1300° C., the briquettes will not melt together. The briquettes which are to be coked according to the present invention may contain any desired binding agent, including water soluble binding agents.

The second constituent of the mixture which is to be coked according to the present invention, i.e., the fines which preferably will possess a particle size of up to 20 mm. generally will be chosen from coking or slightly coking hard coals with between 14% and 40%, preferably between 18% and 25% or 28% volatile constituents, since a mixture of such fines with the above described briquettes will cause formation of a coherent coke cake which can be easily pressed out of this oven and which, on the other hand can be easily separated into coke briquettes and coke breeze. Particularly the combination of such fines with briquettes which when coked alone will not melt together, and the coking of such mixture in a horizontal by-product oven will give the desired result in a very simple and economical manner. However, when the briquettes which are to be coked formed of slightly coking coal or contain a high proportion of pitch or tar, particular care has to be taken in choosing the fine hard coal in order to avoid a mixture which upon coking will possess too strong an adherence between briquette and fines thus making the separation of the coke briquettes from the coke breeze unnecessarily difficult. It is therefore desirable to pre-test the fines which are

to be admixed to the briquettes prior to coking of the thus-formed mixture in order to determine whether the desired result, namely a cake which is easily separable into coke briquettes and coke breeze will be obtained thereby. Anthracite and open burning gas coals should not be used as fines.

The following test has been found to determine accurately the suitability of given fines.

#### TEST I

Cylindrical briquettes are produced of coal and tar, each having a diameter of about 100 mm. and a height of between about 40 and 50 mm. These briquettes are inserted into a crucible made of heat resistant sheet metal and having an inner diameter which is slightly greater than the diameter of the briquettes. The height of the crucible is about 150 mm.

The fines which are to be tested are then poured onto the briquette in the crucible. These fines may be a mixture of fines of different qualities. The crucible is filled in this manner nearly to but not completely to its upper rim in such a manner that the upper face of the layer of fines will be about 1 cm. below the upper rim of the crucible. The cover is then placed on the crucible and the same is embedded in a mass of pulverulent coke having a particular size of less than 5 mm. located in a considerably larger crucible. The larger crucible with the smaller crucible therein is now placed into an electrically heated furnace and heated therein to a temperature of 1000° C. in such a manner that the increase in the temperature equals about 1° C. per minute. Thereafter, the crucibles and the contents thereof are allowed to cool and the coke formed in this manner is then tested as follows:

When it is possible to separate the coke formed of the layer of fines without difficulties from the coked briquette, then the fines or fines mixture are suitable for use in the present method of simultaneously producing coke briquettes and coke breeze. In the opposite case, i.e., when the coke formed of the fines is not easily and without application of substantial force separated from the coke briquette, then it will be necessary to use less-coking fines or to mix coke breeze to the fines or to otherwise reduce the coking characteristics of the mixture of fines, until repetition of the above described test gives the desired result.

The granulation of the fines depends to some extent on the size of the briquettes with which the fines are to be mixed. In order to obtain best utilization of the coke oven space, the particle size of the fines will be up to about 5 mm. when the same is to be coked together with commercial egg-shaped briquettes having diameters of between about 50 and 80 mm. With increasing size of the briquettes, it is also possible to use fines of larger particle size or fines containing a larger percentage of particles of larger size. On the other hand, with diminishing size of the briquettes it is also desirable to use fines of relatively small particle size.

As indicated above, the size of the fines particles is adjusted to the size of the briquettes primarily in order to obtain best possible utilization of the coke oven. By suitably correlating the particle size of the fines to the size of the briquettes, a substantially complete filling of the interspaces between the briquettes with fines particles will be achieved. The foregoing, however, is not to be understood as a limitation of the present invention to specific sizes or size relationships of briquettes and fines. It is also possible to form a mixture of briquettes of varying sizes and of fines of varying particle sizes and composition and to coke the thus-formed mixture in accordance with the present invention.

It is preferred according to the present invention to fill the interspaces between the briquettes by first introducing the briquettes into the coke oven and thereafter allowing the fines to flow or trickle through the inter-

spaces of the mass of briquettes. It is also possible to form in similar manner the mixture of briquettes and fines in a hopper rather than in the coke oven and to introduce the completed mixture of briquettes and fines into the coke oven. If as coking oven a horizontal by-product oven is to be used, then the hopper or the like may be adapted to serve as hopper car for introducing the mixture into the coke oven. When the coking is to be carried out in a continuously operating vertical coking chamber, then it is preferred to refill or fill up the coking chamber by first introducing briquettes and thereafter to allow the fines to flow downwardly through the interspaces between the individual briquettes.

According to the above described preferred manner of carrying out the present invention, namely by first forming a mass of briquettes and then allowing the fines to trickle through the interspaces between the individual briquettes of the mass, the coked end product will be easily divided into briquetted coke and coke breeze. The coke breeze generally can be separated from the briquettes without using special mechanical force, simply by passing the mass over a screen of suitable mesh width so that the briquettes will not fall through the openings in the screen. When relatively larger quantities of fines are mixed with briquettes so that the volume of the fines is more than the volume required for filling the interspaces between the individual briquettes of the mass, then a somewhat coarser coke is obtained in addition to the coke briquettes. However, even in such case, it is very simple to separate the briquettes from the remaining coke and to reduce the particle size of the remaining coke. It is therefore desirable to choose fines which will give a relatively soft coke or a coke which can be easily broken up into smaller particles.

It is a particular advantage of the above described method of the present invention that it is possible in accordance therewith to produce coke briquettes in horizontal by-product ovens which are much more frequently available than vertical coking chambers of which only relatively few are in operation.

Thus, according to the present invention existing installations can be used in order to supply the increasing demand for coke briquettes. Briquetted coke or coke briquettes can be advantageously used for many purposes, for instance in shaft lime kilns, cupola furnaces and blast furnaces. There is particularly great demand for coke briquettes containing between 1 and 10% or preferably between 2 and 6% of volatile constituents since such not completely de-gassed coke briquettes are also eminently suitable for home heating purposes. The desired incomplete coking is accomplished without difficulty either by reducing the coking time or by reducing the coking temperature to between 500 and 900° C.

The simultaneous production of coke breeze, in addition to the coke briquettes is a further important advantage of the new method. Such coke breeze with particle sizes of up to about 10 mm. are obtained only in relatively small quantities, up to about 5% in the conventional coking of hard coal. However, the demand for coke breeze is steadily increasing for various industrial uses for instance in the cement industry or in various sinter methods of ore dressing. It is also possible to incorporate the coke breeze into briquettes which are then treated as described above so as to form coke briquettes. In this manner, by recycling the coke breeze, the only finished product which will be eventually obtained will be coke briquettes.

Good results were obtained by using in accordance with the present invention briquettes which were formed of coke plus about 12% tar; anthracite plus about 10% tar; lean coal containing up to about 14% volatile constituents plus about 8% tar; slightly coking bituminous coals containing about 14%-18% volatile constituents plus about 5% tar; open-burning coal with more than 40% volatile

constituents plus about 7% tar; or, coking coals together with coke or anthracite or the like plus 7% tar.

The second constituent of the mixture which is to be coked as described above, namely the fines, preferably will be a coking hard coal containing between 14 and 40% or most preferably between 18 and 28% of volatile constituents. Anthracite and open-burning coals are not well suited as the fines constituents for the reason that these last named coal types generally will not form a coherent coke cake.

As pointed out further above, when it is desired to form coke briquettes on the one hand and coke breeze on the other hand, the fines should be of a type which will produce a soft, easily comminutable coke and of not too strong coking characteristics.

The embodiments of the present invention described hereinabove are further illustrated in the following examples, the invention however not being limited to the specific details of these examples.

#### Example I

Lean coal containing 13% of volatile constituents and having a particle size of up to 5 mm. is mixed with 7% tar having a softening point of 66° C. (according to Kraemer-Sarnow) and the thus formed mixture is compressed into egg briquettes and placed into a hopper car. A mixture consisting of equal parts of coke breeze having a particle size of up to 5 mm. and open burning coal containing 32% of volatile constituents and also having a particle size of up to 5 mm. is then added to the briquettes and allowed to flow into the interspaces therebetween so as to substantially fill the same. Approximately 30% of the thus formed mixture will be represented by the mixture of coke breeze and open burning coal and about 70% by weight will be represented by the briquettes. The thus formed mixture is then introduced into the coke oven and coked therein for 24 hours at 1200° C. Thereafter, the coke cake is pressed out of the oven in any conventional manner, extinguished and passed over a vibrating screen. Thereby approximately 60% by weight of coke briquettes and 40% by weight of coke breeze are obtained.

#### Example II

45 Coke breeze such as is obtained according to the method of Example I is compressed together with 12% tar and 3% coal tar oil into elliptic briquettes and the thus formed briquettes are introduced into the coke oven. Thereafter, a bituminous coal containing 24% of volatile constituents and having a particle size of up to 10 mm. is introduced from above into the coke oven and allowed to flow down so as to fill the interstices between the previously introduced briquettes. After coking for 20 hours 50 at 1250° C., the thus formed coke cake is pressed out of the coke oven in conventional manner, extinguished and passed over a vibrating screen. In this manner, approximately 65% by weight of coke briquettes and 35% by weight of coke breeze are obtained.

#### Example III

A mixture consisting of equal parts by weight of sub-bituminous coal containing 14% volatile constituents and anthracite containing 6% volatile constituents is 65 pressed with 8% tar into cubes having an edge length of 100 mm. The thus formed briquettes are then mixed with one-half of their weight of a mixture consisting of 70% anthracite and 30% of coking coal containing 20% volatile constituents which mixture has an average particle size of between 1 and 8 mm. Upon coking for 22 hours at 1000° C. a coke cake is obtained which is conventionally removed from the coke oven, extinguished and passed over a vibrating screen. 65% by weight of coke briquettes and 35% by weight of coke breeze are thus obtained.

7  
*Example IV*

A non-coking open burning coal containing 42% of volatile constituents is mixed with 7% of 50% sulfite waste liquor and 7% of hard pitch having a softening point of 155° C. according to Kraemer-Sarnow and the mixture is pressed into egg-shaped briquettes. The thus formed briquettes are mixed with 50% of their own weight of a mixture consisting of 68% of a non-coking open burning coal and 32% of a slightly coking open burning coal. The entire mixture is coked at 1200° C. for 24 hours and then removed from the coke oven and extinguished in conventional manner. After passing the thus formed coke mass over a vibrating screen, the same is separated into about 65% of coke briquettes and 35% of coke breeze.

8  
*Example V*

A finely ground slightly coking coal having 15% of volatile constituents is compressed at 3000 atmospheres into cylindrically shaped briquettes. The thus formed briquettes are then mixed with 50% of their own weight of a mixture consisting of 50% coke breeze and 50% of a coking coal containing 29% volatile constituents. The thus formed mixture is then coked for 18 hours at 900° C., removed from the coke oven, and extinguished and passed over a vibrating screen. 65% of coke briquettes and 35% of coke breeze are obtained.

According to another embodiment of the present invention, a coke is produced the individual pieces of which consist of integral portions some of which have an apparent density of between about 0.7 and 1.1 and others of between about 1.1 and 1.5.

This novel type of coke is produced according to the present invention by coking a mixture of bituminous coal and coal briquettes which when coked alone would only superficially or not at all melt together. In this manner, it is possible according to the present invention to obtain pieces of coke in which the coked coal briquettes are substantially unchanged and present in their initial shape, however, after coking there will be integral with the coke portion which originated from a briquette also a coke portion which originated from the admixture of bituminous fines. Thus, the coke pieces formed in this manner will possess for instance a core portion of greater density than the density of the coke portion surrounding the core. The process can be controlled so that substantially each piece of coke produced thereby consists of portions of higher and portions of lower apparent density, however, it is also possible depending on the degree of admixture of bituminous coal to the coal briquettes, to obtain a coke which also includes coke briquettes which are free of the adherence of any coke originating from the admixture of the bituminous coal. Similarly, it is not necessarily so that the briquette portion of the composite coke piece will be found in the center of the coke piece. It is also possible that such briquette coke portion is only partially covered with coke originating from bituminous coal portion.

In order to determine whether given fines when coked together with coal briquettes will give the desired result, namely coke pieces which possess portions of higher and portions of lower apparent density which portions are integral with each other, it has been found advantageous to carry out tests such as Test I described further above.

This coke formed according to Test I should then be tested to determine whether the fines which had been poured on top of the briquettes are firmly baked to the briquette and also whether shrinkage cracks continue from the fines portion directly into the briquette and vice versa. If this is the case, then it can be assumed that the fines will give the desired result in large-scale coking operations. However, in order to further test this feature, it is suggested to drop the coke piece which has been formed in the inner crucible and which consists of fines and of the briquette from a height of about 2 m. onto a steel

plate. The coke piece will break and examination of the inner surfaces exposed by such fracture of the entire coke piece should show that these fracture surfaces are not identical with the initial boundary surface between the briquette and the fines. The surface exposed by fracture of the coke block should run at an angle to the initial boundary face. In this manner, it can be easily determined that the coke formed of the briquette and the coke formed of the fines have been firmly bound to each other so as to form an integral coke body comprising portions the density of which is controlled by the properties of the coked briquette and portions the density of which is controlled by the properties of the coked fines. If the desired result is not achieved in such tests, then it will become necessary to suitably change the composition of the fines, primarily in the direction of increasing the coking properties thereof.

The dimension of the coal briquettes which form part of the mixture which is subjected to coking according to the present invention will depend on the dimensions of the coke oven and also on the required size of the finally obtained coke pieces. Thus, briquettes of the size of conventional egg briquettes, i.e., having diameters of between about 50 and 80 mm., may be used or also smaller briquettes, for instance such having diameters of between 20 and 50 mm., or also larger briquettes which have diameters greater than 80 mm.

Obviously, the present invention is not limited to the use of briquettes of any given size or of fines of any given particle size. It is also possible to coke in accordance with the last discussed embodiment of the present invention mixtures of briquettes and fines wherein briquettes and/or fines include pieces of varying dimensions.

The proportion of briquettes in the mixture which is to be coked according to the last discussed embodiment of the present invention will depend on the final use of the thus produced coke. For instance, for use as blast furnace coke it will be advantageous to use between about 5 and 30% by weight of briquettes mixed with between 95 and 70% of fines. On the other hand, for use in cupola furnaces, preferably between 30 and 50% by weight of briquettes will be mixed with between 70 and 50% by weight of fines.

It has been suggested previously to operate blast furnaces and cupola furnaces with mixtures of coke briquettes and ordinary coke and to introduce such mixtures into the respective furnaces, whereby, however, the briquettes and the ordinary particulate coke had to be produced separately in accordance with conventional methods. In contrast thereto, according to the present invention, it is now possible to produce coke pieces of varying density and to introduce a single material into the furnace which will contain substantially in each individual piece thereof a portion of coked briquette and of coked fines, i.e., portions of varying density. This represents a considerable technological advance and greatly facilitates the operation of the furnace. It is a further advantage of the last discussed embodiment of the present invention that a single coke oven will suffice to produce the entire coke for the furnace operation while according to conventional methods two types of coke ovens will be required since it is not possible to coke briquettes per se in the conventional horizontal by-product ovens. Generally, for coking briquettes it is necessary to resort to vertical coking chambers of which only relatively few are available while in contrast thereto, horizontal by-product ovens can be found in many installations. These horizontal by-product ovens are entirely sufficient for producing the coke of varying density according to the present invention.

The present invention will also serve to solve the problem of using non-coking or only slightly coking coals in the production of coke. Furthermore, the last discussed embodiment will also permit to incorporate the relatively low coking constituents into the briquettes and

thereby to retain only high cooking fines for the fines portion of the coking mixture. By proceeding in this manner, a greater proportion of low coking or non-coking coal can be introduced into the coke oven than was hereto possible.

The zones or portions of varying apparent density in the individual coke pieces produced according to the last discussed embodiment of the present invention are immediately apparent for instance in microphotographs of polished coke surfaces made of coke pieces produced as described hereinabove. For instance, it may be seen that the relatively dense portion of the coke piece which originated from the briquette will have a relatively low volume such as about 30% and a higher apparent density of about 1.4 while integral therewith and directly adjacent thereto, portions will be found which originated from the fines and which possess a pore volume of about 50% and a corresponding low apparent density of about 0.9.

The following examples will serve to further illustrate the last discussed embodiment of the present invention without however, limiting the invention to the specific details of the examples.

#### Example VI

Lean coal containing about 13% of volatile constituents is compressed into nut-sized briquettes and is then mixed with 4 times its own weight of coking fines containing 20% of volatile constituents. The thus formed mixture is then coked for 24 hours at 1250° C. and thereafter removed from the coke oven and extinguished in conventional manner. The thus produced coke pieces will consist of portions having an apparent density of 0.7 to 0.9 and integral therewith of portions having an apparent density of between 1.3 and 1.5.

#### Example VII

A mixture consisting of 78% lean coal containing 12% volatile constituents, 15% fat coal containing 22% volatile constituents and 7% tar is compressed into egg briquettes and then mixed with 6 times its weight of fat coal containing 26% volatile constituents. The thus formed mixture is then poured into a coking chamber and is coked for 24 hours at a temperature of 1000° C. The coke pieces resulting therefrom are similar to those obtained according to Example VI.

#### Example VIII

Anthracite containing 8% volatile constituents is mixed with 10% tar and then compressed into egg briquettes. The thus formed briquettes are then mixed with twice their own weight of a highly coking coal containing 27% of volatile constituents. The thus formed mixture is then introduced into the coke oven and coked for 24 hours at 1150° C. The coke pieces obtained therefrom possess integral portions of varying density and are particularly suitable for use in the operation of cupola furnaces.

#### Example IX

Finely ground fat coal containing 22% volatile constituents is compressed at a pressure of 3000 atmospheres into cylindrical briquettes and the thus formed briquettes are then mixed with 5 times their own weight of fat fines containing 26% of volatile constituents. The mixture is coked for 22 hours at a temperature of 1150° C. and it will be found that the resulting coke pieces possess integral portions of varying density substantially like those described in connection with Example VI.

The drawing shows a microphotograph of a piece of coke produced in accordance with Example VI. The areas of greater and lesser density are readily apparent.

Without further analysis, the foregoing will so fully reveal the gist of the present invention that others can by applying current knowledge readily adapt it for various applications without omitting features that, from the

standpoint of prior art, fairly constitute essential characteristics of the generic or specific aspects of this invention and, therefore, such adaptations should and are intended to be comprehended within the meaning and range of equivalence of the following claims.

What is claimed as new and desired to be secured by Letters Patent is:

1. A method of producing coke briquettes, comprising the steps of forming a mixture of carbonaceous briquettes which are adapted to be coked without melting together when heated under exclusion of air to between 500° and 1300° C. and of low baking fine hard coal; coking said mixture so as to transform said briquettes and said fines into coke bodies adhering to each other but slightly; and separating the thus-formed coked briquettes from the coked fines so as to obtain coked breeze in addition to and separated from said coke briquettes.
2. A method of producing coke briquettes, comprising the steps of forming a mixture of binder-containing coal briquettes which are adapted to be coked without melting together when heated under exclusion of air to between 500° and 1300° C. and of low baking fine hard coal; coking said mixture so as to transform said briquettes and said fines into coke bodies adhering to each other but slightly; and mechanically separating the thus-formed coked briquettes from the coked fines so as to obtain coke breeze in addition to and separated from said coke briquettes.
3. A method of producing coke briquettes, comprising the steps of forming a mixture of carbonaceous briquettes which are adapted to be coked without melting together when heated under exclusion of air to between 500° and 1300° C. and of low baking fine fat coal containing between 18 and 28 percent of volatile constituents; coking said mixture so as to transform said briquettes and said fines into coke bodies adhering to each other but slightly; and separating the thus-formed coked briquettes from the coked fines so as to obtain coke breeze in addition to and separated from said coke briquettes.
4. A method of producing coke briquettes, comprising the steps of embedding in a horizontal by-product oven coal briquettes which are adapted to be coked without melting together when heated under exclusion of air to between 500° and 1300° C. in low baking fine hard coal; coking said mixture so as to transform said briquettes and said fines into coke bodies adhering to each other but slightly; and mechanically separating the thus-formed coked briquettes from the coked fines so as to obtain coke breeze in addition to and separated from said coke briquettes.
5. A method of producing coke briquettes, comprising the steps of forming a mixture of carbonaceous briquettes which are adapted to be coked without melting together when heated under exclusion of air to between 500° and 1300° C. and of low baking fine hard coal, the quantity of said fines being so chosen as to be substantially sufficient to fill the interstices between said carbonaceous briquettes; coking said mixture so as to transform said briquettes and said fines into coke bodies adhering to each other but slightly; and separating the thus-formed coked briquettes from the coked fines so as to obtain coke breeze in addition to and separated from said coke briquettes.
6. A method of producing coke bodies of varying density, comprising the steps of forming a mixture of carbonaceous briquettes which are adapted to be coked without melting together when heated under exclusion of air to be between 500° and 1300° C. and of strongly baking bituminous fines; and coking said mixture so as to transform said briquettes and said bituminous fines into coherent coked bodies each of which including portions of relatively high density and integral therewith portions of relatively low density.
7. A method of producing coke bodies of varying density, comprising the steps of forming a mixture of carbonaceous briquettes which are adapted to be coked

without melting together when heated under exclusion of air to be between 500° and 1300° C. and of strongly baking bituminous fines; coking said mixture so as to transform said briquettes and said bituminous fines into a coked body including portions of relatively high density and integral therewith portions of relatively low density; and subdividing said coked body so as to obtain a plurality of smaller coked bodies substantially each of which comprises integral portions of relatively high and relatively low density.

8. A method of producing coke bodies of varying density adapted for use in blast furnace operations, comprising which are adapted to be coked without melting together and 5 percent by weight of carbonaceous briquettes which are adapted to be coked without melting together when heated under exclusion of air to be between 500° and 1300° C. and of between about 70 and 95 percent by weight of strongly baking bituminous fines; and coking said mixture so as to transform said briquettes and said bituminous fines into coherent coked bodies each of which including portions of relatively high density and integral therewith portions of relatively low density.

9. A method of producing coke bodies of varying density adapted for use in cupola furnace operation, comprising the steps of forming a mixture of between about 30 and 50 percent by weight of carbonaceous briquettes

which are adapted to be coked without melting together when heated under exclusion of air to be between 500° and 1300° C. and of between about 70 and 50 percent by weight of strongly baking bituminous fines; and coking said mixture so as to transform said briquettes and said bituminous fines into coherent coked bodies each of which including portions of relatively high density and integral therewith portions of relatively low density.

10. A method of producing coke, comprising the steps of forming a mixture of carbonaceous briquettes which are adapted to be coked without melting together when heated under exclusion of air to be between 500° and 1300° C., and of fine hard coal; and coking the thus formed mixture so as to transform said briquettes and said coal into coke.

#### References Cited in the file of this patent

##### UNITED STATES PATENTS

|           |                |       |                |
|-----------|----------------|-------|----------------|
| 1,824,526 | Andrews        | ----- | Sept. 22, 1931 |
| 2,353,753 | Otto           | ----- | July 18, 1944  |
| 2,600,078 | Schutte et al. | ----- | June 10, 1952  |
| 2,907,698 | Schulz         | ----- | Oct. 6, 1959   |

##### FOREIGN PATENTS

|         |               |       |              |
|---------|---------------|-------|--------------|
| 389,066 | Great Britain | ----- | June 2, 1931 |
|---------|---------------|-------|--------------|